

## UNITED STATES PATENT OFFICE.

THOMAS WILLIAM STAINER HUTCHINS, OF DAVENHAM, NEAR NORTHWICH,  
ENGLAND.

## ELECTRODEPOSITION OF METALS.

No Drawing. Application filed June 30, 1925, Serial No. 40,685, and in Great Britain July 24, 1924.

In the electro-deposition of metals in the form of tubes or sheets, it is usual practice to provide upon the mandrel or former and as the base upon which the deposited metal can grow, a covering or coating of a material or mixture of materials which, whilst having the necessary properties for ensuring a good birth or initiation of deposit, can be readily detached from the latter when deposition is completed by melting so as to allow of the convenient withdrawal or removal of the deposited tube or sheet from the mandrel or former. A usual procedure is to deposit lead or a suitable wax impregnated with graphite or other electrical conducting material upon the mandrel or former and to electrolytically deposit the tubes or sheets upon the lead or graphite-impregnated wax. On the completion of the electro-deposition of the tube or sheet, each mandrel is placed in a furnace or otherwise suitably heated to melt the depositing surface of lead or impregnated wax, when the tube or sheet can be withdrawn or removed from the mandrel or former.

It will be readily understood that the employment of a special depositing surface is a source of expense and such surface is a frequent cause of failure in the electro-deposition. Attempts have been made to provide a metal or alloy from which the mandrel or former can be constructed which will serve for the direct deposition of the metal without the intermediate coating, but as far as I am aware, a commercially successful result has not so far been attained in this direction. It will be appreciated that the metal or alloy used must provide a surface upon which a good birth of deposit can be made, must be insoluble or practically insoluble in the electrolyte and must not have such a degree of attachment to the deposited metal that the latter cannot be removed therefrom by a blow or pressure.

By research and experiment, I have found that a mandrel or former made of an alloy of steel and chromium and/or iron and chromium, after having its surface polished is capable of successful use for the reception of electrolytic deposits of iron and other metals. The percentage of chromium in the alloy can be varied without seriously affecting the properties required of a mandrel or former, and as hereinbefore indicated, but

I find an alloy containing iron and/or steel with from 12 to 14 per cent chromium gives 55 good results.

I have further found that if for a tubular deposit the mandrel has a slight taper, than after depositing the metal thereon, a subsequent annealing and chilling process results 60 in the detachment of the metal from the mandrel.

My invention comprises therefore the improved mandrels, formers or bases for use in the electro-deposition of metals made from 65 an alloy of steel and/or iron and chromium, and having a polished surface.

My invention further comprises the employment in the electro-deposition of cylinders or sleeves of metals, of a tapered mandrel 70 or former made from an alloy of steel and/or iron and chromium.

My invention further comprises the improved process of and means for facilitating the obtaining of metal cylinders or sleeves 75 deposited on mandrels, consisting in depositing the metal on a preferably tapered mandrel made from an alloy of steel and/or iron and chromium, heating the metal and mandrel and then quickly cooling or chilling 80 the metal and mandrel whereby separation of the two is effected.

In one convenient application of the invention to the deposition of metal cylinders or sleeves, the chromium alloy mandrel is 85 made with a small taper and is given a polished surface. The metal is then deposited thereon. The mandrel with the metal thereon is then placed in an annealing furnace and after the requisite temperature for annealing 90 purposes has been reached and maintained for any desired period, the mandrel and metal are lowered into a vat with a cooling fluid therein. The effect of the chilling action is to release the metal from the mandrel.

My improved mandrels or formers gives a good birth of deposit, allow of the ready detachment or removal of the deposited metal tube or sheet therefrom either before or after 100 the annealing process, and are practically insoluble in the electrolyte.

It will be understood that my invention can be applied to formers of disc, ribbon or sheet form which are then made of an alloy 105 of steel and for iron or chromium, the face

of which has been polished. The deposited metal would be removed by pressure or in any other ordinary manner.

I claim:

- 5 1. A process for the electrolytic formation of metals in tubular formation which comprises electrolytically depositing metals on a tubular polished tapered cathode made of an alloy containing a major proportion of iron and a minor proportion of chromium, heating the cathode and deposited metal, then quickly chilling the metal and cathode whereby separation of the formed tube and cathode occurs.
- 10 15 2. A process for the electrolytic formation of iron tubes which comprises electrolytically depositing iron on a tubular polished tapered cathode made of an alloy containing

a major proportion of iron and a minor proportion of chromium, heating the cathode 20 and deposited iron, then quickly cooling the iron and cathode whereby separation of the formed tube and cathode occurs.

3. A process for the electro-deposition of metals which comprises electrolytically depositing a metal upon a polished cathode made of an alloy containing a major proportion of iron and a minor proportion of chromium, heating the cathode and deposited metal, then quickly chilling the metal and 30 cathode whereby separation of the deposited metal and cathode occurs.

In testimony whereof I have signed my name to this specification.

THOMAS WILLIAM STAINER HUTCHINS.